

## UNITED STATES PATENT OFFICE

1,969,737

## ELECTRICAL INSULATING OIL

Seymour W. Ferris, Lansdowne, Pa., assignor to  
The Atlantic Refining Company, Philadelphia,  
Pa., a corporation of Pennsylvania

No Drawing. Application January 16, 1931,  
Serial No. 508,004

7 Claims. (Cl. 196—13)

The present invention relates to improvements in mineral oil compositions, and has particular reference to the production of improved oils for use in connection with electrical equipment, as 5 an insulating and/or cooling medium.

The reason for the use of insulating oils in electrical equipment such as capacitors, transformers, and cables is primarily based upon the fact that these oils have a greater resistance to electrical 10 potential than does air, for example. With different types of apparatus and under varying conditions of use, insulating oils may have a range of viscosities varying, for example, between 50 seconds Saybolt Universal at 100° F. and 200 15 seconds Saybolt Universal at 210° F. The value of any particular insulating oil depends upon its electrical qualities, in particular, its resistance to the flow of an electric current therethrough. This quality is known in the art as "resistivity", 20 and is customarily measured in meg. meg. ohms per cm.<sup>3</sup>, according to A. S. T. M. method D-257-29T.

Electrical oils have been developed, in accordance with the prior art, which have a satisfactory initial resistivity; but upon being subjected to use in electrical equipment over an extended period of time it is characteristic of the prior art oils that they lose their high resistivity or break down. In order to determine in advance the 25 resistivity-stability of a particular oil or how long it will stand up in actual use in electrical equipment, there has been developed an oxidation test, which is accepted as approximating extended operating conditions. This method consists in placing 100 gms. of the oil to be tested into a 30 250-330 cc. Pyrex Erlenmeyer flask, closing the mouth of the flask with a cork stopper perforated or slotted so that a free circulation of air may be maintained over the oil, and immersing the flask in an oil bath maintained at 100° C., allowing 35 it to remain in such bath for 72 hours. After this time the oil sample is removed from the bath and its resistivity measured at 85° C. in accordance with the A. S. T. M. method D-257-29T. A 40 comparison of the results of this test with its initial resistivity constitutes a means for evaluating the resistivity-stability of an oil.

A primary object of the present invention is the production of oils which have a higher resistivity-stability than oils known heretofore, and more specifically oils which will not substantially decrease in resistivity or which will remain of substantially the same resistivity for prolonged periods of time, or which may, in fact, after actual use and/or when subjected to the aforesaid test

show a final resistivity greater than their initial resistivity.

In my copending application, Serial Number 206,388 filed July 16, 1927, which on January 13, 1931, issued as U. S. Patent No. 1,788,569, of which the present application is a continuation in part, there is described a process for separating an oil into constituents which are respectively more paraffinic and more naphthenic, by extraction of the latter type of constituents from the original 65 oil with an aromatic nitro compound such as nitrobenzene. The various series of hydrocarbons which comprise mineral oils possess a differential solubility in nitrobenzene, naphthenic compounds being more soluble therein than paraffinic compounds. 70

I have found that by a modification of this process I am able to produce insulating oils having novel characteristics with respect to resistivity-stability. A petroleum oil, for example, 75 a refined distillate, is divided into a number of fractions by extraction with nitrobenzene. Each extraction is preferably made by heating one part of oil with two parts of nitrobenzene to miscibility, cooling the mixture to 10° C., whereby 80 a two layer system is formed on settling, separating the layers, and removing nitrobenzene from each fraction. The operation is then repeated on the nitrobenzene undissolved fraction 85 any desired number of times. These various fractions, particularly after treatment with fuller's earth, behave differently with respect to resistivity-stability. Certain of the fractions, for example, the first dissolved fraction will act somewhat as the insulating oils known heretofore, that is, will show a pronounced decrease in resistivity 90 after being subjected to the aforesaid oxidation test or after equivalent use in electrical apparatus. However, other fractions will act in a manner entirely unknown in the prior art, that is, certain of these fractions will show an increase in resistivity upon actual use or when subjected to 95 said oxidation test. The fraction or fractions which have this novel characteristic of increasing in resistivity will depend upon such factors as the particular oil and conditions under which the extraction and clay treatment are effected. 100

My invention will be more specifically explained in the following examples:

105

## Example I

A pipe still residuum from a Mid-Continent pressed paraffin distillate, having been subjected 110

to acid treatment in the amount of 14 lbs. of 66° Bé.  $H_2SO_4$  per barrel of oil and a subsequent contact clay treatment, was employed as a starting material. This refined oil had a viscosity of 284 seconds Saybolt Universal at 100° F., and a gravity of 25.0° A. P. I. 100 parts of the oil was heated with 50 parts of nitrobenzene to complete miscibility. This mixture was then cooled to 10° C. and settled, whereby a two layer system comprising a lower layer of nitrobenzene dissolved oil and an upper layer of nitrobenzene undissolved oil was formed. The two layers were separated, by decanting, and the two oil fractions freed from nitrobenzene by vacuum distillation. 80.7 parts of nitrobenzene undissolved oil resulted and this was heated to miscibility with 75 parts of nitrobenzene, and the mixture treated as before. An additional extraction was made upon the 63 parts of nitrobenzene undissolved fraction resulting from the second extraction, 150 parts of nitrobenzene being employed. From this third extraction was recovered 30.7 parts of undissolved oil. After being freed from nitrobenzene the first, second and third nitrobenzene dissolved fractions and the final undissolved oil were percolated through finely divided fuller's earth at a temperature of approximately 70° C. Initial electrical resistivity tests were made upon each oil fraction, after which the fractions were subjected to the oxidation test aforementioned, and final resistivities taken. The results may be tabulated as follows:

| 35 | Percent by vol.       | Clay yield bbls. per 17 ton | Sp. grav. 15.5° C. | Vis. @ 100° F. | Resistivity @ 85° C. |                          |
|----|-----------------------|-----------------------------|--------------------|----------------|----------------------|--------------------------|
|    |                       |                             |                    |                | Init.                | After 72 hours @ 100° C. |
| 40 | Dissolved Fract. #1   | 19.3                        | 243                | .9371          | 457                  | 4.0                      |
|    | Dissolved Fract. #2   | 27.7                        | 243                | .9279          | 368                  | 10.6                     |
|    | Dissolved Fract. #3   | 22.1                        | 243                | .8973          | 255                  | 30.8                     |
|    | Undissolved Fract. #3 | 30.7                        | 243                | .8623          | 176                  | 5.52                     |
|    |                       |                             |                    |                |                      | 28.4                     |

45 It will be noted that the nitrobenzene undissolved fraction No. 3 has an initial electrical resistivity of 5.52 meg. meg. ohms per  $cm.^3$  which increases after being subjected to the oxidation test to 28.4 meg. meg. ohms per  $cm.^3$  This particular fraction makes a highly desirable insulating oil for commercial use in electrical instruments. The remaining fractions exhibit a drop in resistivity which is characteristic of insulating 55 oils known heretofore.

#### Example II

A distillate from an acid-treated Mid-Continent crude oil was filtered through fuller's earth, to produce a refined oil having a viscosity of 163 seconds Saybolt Universal at 100° F., and a specific gravity of 0.8905 at 15.5° C. This oil was subjected to two extractions with nitrobenzene, in each extraction employing two parts of nitrobenzene to one part of the original oil. The first and second nitrobenzene soluble fractions and the final nitrobenzene undissolved oil, after being freed from nitrobenzene, were filtered through finely divided fuller's earth at approximately 75° C. Upon determining the initial electrical resistivity of each, the filtered fractions were subjected to the oxidation test above set forth, after which final resistivity determinations

were made. The results may be tabulated as follows:

|                      | Yield percent by vol. | Clay yield bbls. per 17 ton | Sp. grav. 15.5° C. | Vis. @ 100° F. | Resistivity @ 85° C. |                          |
|----------------------|-----------------------|-----------------------------|--------------------|----------------|----------------------|--------------------------|
|                      |                       |                             |                    |                | Original             | After 72 hours @ 100° C. |
| Original             |                       |                             |                    |                | 80                   |                          |
| 1st soluble fraction | 36.0                  | 220                         | .8905              | 163            | 13.1                 | 1.07                     |
| 2nd soluble fraction | 27.5                  | 177                         | .9230              | 230            | 4.5                  | 2.0                      |
| Undissolved fraction | 35.7                  | 194                         | .8827              | 184            | 20.0                 | 33.4                     |
|                      |                       |                             |                    |                | 85                   |                          |
| Original             |                       |                             |                    |                | 90                   |                          |
| 1st soluble fraction | 36.0                  | 220                         | .8581              | 135            | 50.0                 | 3.7                      |

With this particular oil and under the conditions of treatment, it is seen that the second nitrobenzene dissolved fraction exhibits an increase in electrical resistivity after being subjected to the oxidation test.

#### Example III

100 parts of a Pennsylvania distillate having a viscosity of 307 seconds Saybolt Universal at 100° F., and a gravity of 29.4° A. P. I. was subjected to eight extractions with nitrobenzene, each extraction being made by heating 200 parts of the solvent with the undissolved residue from the last extraction to obtain miscibility and cooling to effect the formation of a two-layer system. Dissolved fractions 4 and 5 were mixed as were 105 dissolved fractions 6, 7, and 8. After being freed from nitrobenzene by vacuum distillation and clay filtered at 75° C., the fractions were subjected to the oxidation test, resistivity determinations being made before and after said test.

|                               | Percent by vol. | Clay yield bbls. per 17 ton | Sp. grav. 15.5° C. | Vis. @ 100° F. | Resistivity @ 85° C. |                          |
|-------------------------------|-----------------|-----------------------------|--------------------|----------------|----------------------|--------------------------|
|                               |                 |                             |                    |                | Init.                | After 72 hours @ 100° C. |
| Dissolved fraction #1         | 27.5            | 243                         | .9213              | 648            | .862                 | 2.43                     |
| Dissolved fraction #2         | 16.0            | 243                         | .8833              | 321            | .822                 | 13.3                     |
| Dissolved fraction #3         | 11.6            | 243                         | .8682              | 243            | .816                 | 52.3                     |
| Dissolved fraction #4, #5     | 20.8            | 243                         | .8592              | 223            | .796                 | 61.8                     |
| Dissolved fraction #6, #7, #8 | 21.6            | 243                         | .8509              | 216            | .786                 | 75.8                     |
|                               |                 |                             |                    |                | 110                  |                          |
| Dissolved fraction #1         |                 |                             |                    |                | 111                  |                          |
| Dissolved fraction #2         |                 |                             |                    |                | 112                  |                          |
| Dissolved fraction #3         |                 |                             |                    |                | 113                  |                          |
| Dissolved fraction #4, #5     |                 |                             |                    |                | 114                  |                          |
| Dissolved fraction #6, #7, #8 |                 |                             |                    |                | 115                  |                          |

As will be recognized by one skilled in the art of an oil which increases in electrical resistivity upon being subjected to conditions which cause a substantial decrease in the resistivity of oils known heretofore, constitutes a considerable improvement in the art. I am unable to explain why the oils produced according to my process exhibit this novel characteristic. Regardless of theory, however, I have found that these oils are highly desirable for use as an insulating and/or cooling medium in electrical equipment.

While my invention has been described somewhat specifically, it is intended to include modifications coming within the spirit thereof and as defined by the appended claims.

What I claim is:

1. A process for producing insulating oils, which comprises separating a viscous petroleum oil into a number of fractions by extraction with nitrobenzene, removing the nitrobenzene from said fractions, contacting said fractions with a solid adsorptive agent, thereafter removing said agent therefrom, and selecting for use as insulating oils, those fractions, samples of which upon being subjected to a temperature of 100° C. 14

- for 72 hours, show no substantial decrease in electrical resistivity.
2. For use as an electrical insulating medium, an oil produced by the extraction of a viscous mineral oil with nitrobenzene, which upon being maintained at 100° C. for 72 hours, exhibits substantially no decrease in electrical resistivity.
3. For use as an electrical insulating medium, an oil produced by the extraction of a viscous mineral oil with nitrobenzene, which, upon being maintained at 100° C. for 72 hours, exhibits an increased electrical resistivity.
4. In the production of insulating oils, the steps which comprise separating viscous petroleum oil into fractions by solvent extraction, removing the solvent from the soluble and insoluble fractions maintaining samples of the fractions at a temperature of 100° C. for 72 hours, and selecting those fractions, samples of which show no substantial decrease in electrical resistivity after being subjected to said temperature for said time, for use as insulating oils.
5. An electrical insulating oil prepared by extracting a viscous mineral oil with a solvent and separating the solvent from the fractions resulting, said insulating oil, upon maintaining a sample thereof at 100° C. for 72 hours, showing no substantial decrease in electrical resistivity. 80
6. An electrical insulating oil comprising a viscous mineral oil having, when measured at 85° C. in accordance with A. S. T. M. D-257-29T, an electrical resistivity of at least 5 meg. meg. ohms per cm.<sup>3</sup>, which upon being maintained at a temperature of 100° C. for 72 hours, exhibits substantially no decrease in electrical resistivity. 85
7. An electrical insulating oil comprising a viscous mineral oil having, when measured at 85° C. in accordance with A. S. T. M. method D-257-29T, an electrical resistivity of at least 5 meg. meg. ohms per cm.<sup>3</sup>, which upon being maintained at a temperature of 100° C. for 72 hours, exhibits an increase in electrical resistivity. 90
- 95

SEYMOUR W. FERRIS.

|    |     |
|----|-----|
| 25 | 100 |
| 30 | 05  |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |